



US010351284B2

(12) **United States Patent**  
**Niedersuess et al.**

(10) **Patent No.:** **US 10,351,284 B2**  
(45) **Date of Patent:** **Jul. 16, 2019**

(54) **COLLATION SHRINK FILMS**

(71) Applicant: **Borealis AG**, Vienna (AT)

(72) Inventors: **Peter Niedersuess**, Riedmark (AT);  
**Minna Aarnio-Winterhof**, Altenberg  
(AT)

(73) Assignee: **Borealis AG**, Vienna (AT)

(\*) Notice: Subject to any disclaimer, the term of this  
patent is extended or adjusted under 35  
U.S.C. 154(b) by 830 days.

(21) Appl. No.: **14/395,089**

(22) PCT Filed: **Apr. 17, 2013**

(86) PCT No.: **PCT/EP2013/058020**

§ 371 (c)(1),  
(2) Date: **Oct. 17, 2014**

(87) PCT Pub. No.: **WO2013/156532**

PCT Pub. Date: **Oct. 24, 2013**

(65) **Prior Publication Data**

US 2015/0076022 A1 Mar. 19, 2015

(30) **Foreign Application Priority Data**

Apr. 18, 2012 (EP) ..... 12164652

(51) **Int. Cl.**

**B65B 11/58** (2006.01)  
**B65B 21/24** (2006.01)

(Continued)

(52) **U.S. Cl.**

CPC ..... **B65B 53/02** (2013.01); **B65B 11/58**  
(2013.01); **B65B 21/245** (2013.01); **B65B**  
**27/04** (2013.01); **B65D 71/08** (2013.01);  
**B65D 71/10** (2013.01)

(58) **Field of Classification Search**

CPC ..... B65B 11/58; B65B 13/02; B65B 27/04;  
B65B 53/02; B65D 71/08

(Continued)

(56) **References Cited**

U.S. PATENT DOCUMENTS

3,062,373 A \* 11/1962 Reynolds ..... B65D 71/10  
206/160

3,417,540 A \* 12/1968 Copping ..... B65B 35/36  
198/419.3

(Continued)

FOREIGN PATENT DOCUMENTS

EP 0 299 750 A2 1/1989  
EP 0 380 353 A2 8/1990

(Continued)

*Primary Examiner* — Gloria R Weeks

*Assistant Examiner* — Patrick B Fry

(74) *Attorney, Agent, or Firm* — Eversheds Sutherland  
(US) LLP

(57) **ABSTRACT**

A process for collation shrink wrapping an object that may include a number of individual containers, preferably a number of substantially identical containers. The process may include the steps of (i) obtaining a binding tape that is a film uniaxially oriented in the machine direction (MD) and wrapping the tape around the object, (ii) sealing the ends of the now wrapped binding tape (i.e., to form a loop), (iii) obtaining a collation shrink film that may include a multi-modal linear low density polyethylene (LLDPE), the film being a stretched film that is uniaxially oriented in the machine direction (MD) in a draw ratio of at least 1:3, (iv) wrapping the collation shrink film around the object of step (ii), (v) heating the wrapped object of step (iv) such that the tape shrinks in its machine direction and the collation shrink film shrinks in its machine direction.

**11 Claims, 2 Drawing Sheets**



\* cited by examiner



FIG. 1



FIG. 2



*FIG. 3*

## COLLATION SHRINK FILMS

This invention relates to collation shrink process, in particular a collation shrink process which employs a multimodal linear low density polyethylene film that has been uniaxially stretched in the machine direction. In particular, the process involves the use of a uniaxially oriented film as above and a binding tape formed from a uniaxially oriented film to collation shrink wrap an object. The invention also provides an object shrink wrapped using the process of the invention.

## BACKGROUND OF THE INVENTION

Collation shrink films are films that are wrapped around an object to be packaged and shrunk to keep the units within the object together. The most common use of these films is in the packaging of multiple containers, such as bottles or cans which might contain food, beverages and so on. The collation shrink film is wrapped around a number of the containers, perhaps a 6-pack of drinks or 24 pack of food cans held in a cardboard base and shrunk around the containers. The skilled person is familiar with this rapidly expanding film area.

The wrapping process typically involves a shrink oven or shrink tunnel in which the film and object covered by the film is briefly heated to cause the collation shrink wrapping to occur. The plastic film then collapses around the multiple containers and holds the units in place.

Films which are used as collation shrink films obviously need to possess certain properties to make them commercially interesting. Some of the main characteristics that are required for film applications in this market segment are good shrinkage. The films must possess excellent strength after shrinkage, often referred to as load retention resistance. This property requires that films are stiff.

Films must resist puncture and must not be sticky. The consumer does not want the packaged product to stick to the film. The collation shrink films are cut during the wrapping process so the ability to be cut is important.

Sealing properties are also important. During the wrapping process, the two sides of the film are passed around the object being wrapped and are contacted, typically underneath the product being wrapped. These two film edges must be sealed and the seal strength needs to be high. The whole packaged ensemble is often carried simply by grabbing hold of the packaging film. If the seal strength is weak, the film can fail during this operation. The seal strength must ideally be strong enough to hold the weight of the object packaged. Where the object is a 24 pack of tins, for example, the weight can be significant.

Finally, the brand owner of the goods being packaged ideally wants his products to be clearly visible through the packaging. Optical properties such as low haze and high gloss that result in a brilliant print appearance are important.

Low Density Polyethylene (LDPE) currently dominates the collation films market segment with its good shrink behaviour, especially in transverse direction (TD). It is known however, that multimodal LLDPE exhibits significant benefits over LDPE when blended with other linear low density polyethylene and high density polyethylene components. This mixture offers the highest performance on all key shrink parameters for collation shrink films.

Thus, current collation shrink film solutions are polyethylene blown films which are made from LDPE and LLDPE and/or HDPE. The LDPE is necessary to give high shrink

rate and the LLDPE / HDPE component gives a combination of stiffness, toughness and bundling force (also known as cold shrink force).

A major consideration in this rapidly expanding market is costs. Film down-gauging, i.e. using thinner films offers an obvious way of saving costs as thinner films means less film per unit packaged. Down gauged films can only be used however, when the other properties of the film as discussed above are maintained. The mechanical properties in particular need to be maintained.

The present invention targets new collation shrink films that can provide these core properties but preferably down gauged. Today there are polyethylene based blown films for collation shrink applications in use with a thickness of approximately 38-45µm. The present inventors sought films having a thickness (before shrinkage) of less than 38 microns. Ideally, the present inventors sought to down gauge the films to approximately 28 to 32 µm.

One possible route to down gauged films might be to add high density polyethylene (HDPE). The high stiffness of HDPE gives the shrunk film the necessary bundling force, but it makes it necessary to use a higher temperature in the shrink tunnel to effect shrinkage. Moreover, the mechanical strength of the film is poor and the film breaks under stress (e.g. when the bundle is lifted or moved). This solution is not therefore favoured.

Surprisingly, the inventors have found that the use of uniaxially oriented multimodal LLDPE films offers a possible solution to the problem here. When using a monoaxial stretched film of multimodal based LLDPE it is possible to achieve a thin film providing high mechanical strength and high bundling force and at the same time a very high shrink rate/shrink force at significantly lower temperature compared to non oriented blown film.

It is a key feature of this invention that the temperature required to effect shrinkage is much lower than is conventionally used in a collation film shrink tunnel. Lower temperatures mean lower costs and the product being packaged is not exposed to as high temperatures. This minimises the risk of product degradation.

However, the use of uniaxial (machine direction) oriented films and the use of low temperatures during the collation shrink process is limited by the transverse direction shrink of these films. If there is insufficient transverse direction shrinkage then the bundling force of the film can be too low in the transverse direction. Goods packaged using such a film might therefore work their way loose during transport.

The inventors therefore propose the use of a binding tape or binding strip which is also a machine direction uniaxially oriented film, ideally of the same composition as the collation shrink film. This tape can be passed around the object being wrapped in such a way that when it is subjected to heat, the binding tape shrinks in its machine direction around the object. The tape is oriented such that its shrinkage provides bundling force in the transverse direction of the main collation shrink film. The tape needed can simply be cut from the main collation shrink film. The tape might also form a handle for carrying the goods.

It will be appreciated that in any collation shrink wrapping process two ends of the object being wrapped remain open. This provides a potential source of weakness in the collation shrink wrapped object. A further benefit of the use of a binding tape is that this tape will at least partially cover the open end providing additional strength to the package and possibly a kind of handle.

In this way, an object can be shrink wrapped using a potentially down gauged machine direction oriented (MDO)

film at lower temperature than conventional collation shrink films and high bundling forces. This is advantageous in terms of cost and due to the fact that the materials packaged are not subjected to such high temperature.

## SUMMARY OF INVENTION

Viewed from one aspect the invention provides a process for collation shrink wrapping an object which comprises a plurality of individual containers, preferably a plurality of substantially identical containers, comprising:

(i) obtaining a binding tape which is a film uniaxially oriented in the machine direction (MD) and wrapping said tape around said object;

(ii) sealing the ends of the now wrapped binding tape (i.e. to form a loop); (iii) obtaining a collation shrink film comprising a multimodal linear low density polyethylene (LLDPE), said film being a stretched film which is uniaxially oriented in the machine direction (MD) in a draw ratio of at least 1:3;

(iv) wrapping said collation shrink film around said object of step (ii); (v) heating said wrapped object of step (iv) such that the tape shrinks in its machine direction and the collation shrink film shrinks in its machine direction.

In another aspect the invention provides a process for collation shrink wrapping an object which comprises a plurality of individual containers, preferably a plurality of substantially identical containers, comprising:

(i) obtaining a binding tape which is a film uniaxially oriented in the machine direction (MD) and wrapping said tape around said object;

(ii) sealing the ends of the now wrapped binding tape (i.e. to form a loop);

(iii) obtaining a collation shrink film comprising a multimodal linear low density polyethylene (LLDPE), said film being a stretched film which is uniaxially oriented in the machine direction (MD) in a draw ratio of at least 1:3;

(iv) wrapping said collation shrink film around said object of step (ii) in such a way that when said binding tape shrinks in its machine direction upon the application of heat, that direction represents substantially the transverse direction for the collation shrink film;

(v) heating said wrapped object of step (iv) such that the tape shrinks in its machine direction and the collation shrink film shrinks in its machine direction. Said directions are preferably therefore orthogonal.

Viewed from another aspect the invention provides a process for collation shrink wrapping an object which comprises a plurality of individual containers, preferably a plurality of substantially identical containers, comprising:

(i) obtaining a binding tape which is a film uniaxially oriented in the machine direction (MD) and wrapping said tape around said object;

(ii) sealing the ends of the now wrapped binding tape (i.e. to form a loop);

(iii) obtaining a collation shrink film comprising a multimodal linear low density polyethylene (LLDPE), said film being a stretched film which is uniaxially oriented in the machine direction (MD) in a draw ratio of at least 1:3;

(iv) wrapping said film around said object of step (ii) in such a way that when said binding tape shrinks in its machine direction upon the application of heat, that direction represents substantially the transverse direction for the collation shrink film, that direction is perpendicular to the shrinkage of the collation shrink film;

(v) heating said wrapped object of step (iv) such that the tape shrinks in its machine direction and the collation shrink film shrinks in its machine direction.

It will be appreciated that the collation shrink film will be provided on a spool. The process of the invention may therefore involve the steps of dispensing film from said spool and cutting the film into an appropriate length to wrap around said object.

Viewed from another aspect the invention provides an object which comprises a plurality of individual product containers shrink wrapped by the process as hereinbefore defined.

Viewed from another aspect the invention provides a process for a process for collation shrink wrapping an object which comprises a plurality of individual containers, preferably a plurality of substantially identical containers, comprising:

(i) obtaining a collation shrink film comprising a multimodal linear low density polyethylene (LLDPE), said film being a stretched film which is uniaxially oriented in the machine direction (MD) in a draw ratio of at least 1:3;

(ii) cutting a binding tape from said collation shrink film;

(iii) wrapping said tape around said object and sealing the ends of the now wrapped binding tape (i.e. to form a loop);

(iv) wrapping at least a part of said remaining collation shrink film around said object; in a direction such that when said binding tape shrinks in its machine direction upon the application of heat, that direction represents substantially the transverse direction for the collation shrink film;

(v) heating said wrapped object of step (iv) such that the tape shrinks in its machine direction and the collation shrink film shrinks in its machine direction.

## DEFINITIONS

The term LLDPE means linear low density polyethylene herein. The term when exposed to a temperature of 170° C. or less refers to the temperature of the environment around the film such as the temperature of the oven in which the film is placed or the temperature of an oil bath in which the film is placed. It will be appreciated that if the film is present in an oven for a short period of time, the film itself may not heat to the oven temperature. For ease of measurement however, when exposed to a temperature of 170° C. or less refers to that oven temperature and so on rather than the actual film temperature.

The term "an object which comprises a plurality of individual product containers" means that the object being wrapped is itself formed from a plurality of preferably identical containers such as cans, tins, bottles, jars, plastic liquid dispensers (e.g. shower gel, shampoo, and soap containers) and so on. The number of such containers making up the object might vary, e.g. from 4 to 64 containers. The skilled person will be familiar with objects that can be wrapped such as a 6-pack of beverages, 24 pack of food cans and so on.

The product here is not a product formed from a large number of small identical units such as rice, sweets or pasta but is based on a series of containers which contain a desired product.

Often the multiple containers might be carried on a tray, such as a cardboard tray. In that case, the tray forms part of the object being wrapped.

The containers will typically be arranged in a regular pattern such as a square or rectangle. Containers can have any cross-section such as circular (like bottles and cans), oval, square, rectangular or irregular. The smallest cross-

section of any container is preferably at least 2 cm. The maximum cross-section is preferably 30 cm. Containers will not typically be stacked before wrapping. There will preferably be a single layer therefore of containers to be wrapped.

The films of the invention are uniaxially oriented in the machine direction. They are not stretched in the transverse direction. The films of the invention are not therefore biaxially oriented.

#### DETAILED DESCRIPTION OF INVENTION

The collation shrink film of the invention must comprise at least a multimodal LLDPE. It will be appreciated that in any polyethylene of the invention that ethylene forms the major monomer unit present such as at least 80 wt % of the monomer residues present.

It will be preferred if the multimodal LLDPE forms the most abundant polymer present within the film as a whole, i.e. it has the largest weight percentage. Ideally, at least 50 wt % of the collation shrink film is formed from a multimodal LLDPE.

The LLDPE of use in this invention is multimodal. The term "multimodal" means multimodal with respect to molecular weight distribution and includes also therefore bimodal polymers.

Usually, a LLDPE composition, comprising at least two polyethylene fractions, which have been produced under different polymerisation conditions resulting in different (weight average) molecular weights and molecular weight distributions for the fractions, is referred to as "multimodal". The prefix "multi" relates to the number of different polymer fractions present in the polymer. Thus, for example, the term multimodal polymer includes so called "bimodal" polymers consisting of two fractions. The form of the molecular weight distribution curve, i.e. the appearance of the graph of the polymer weight fraction as a function of its molecular weight, of a multimodal polymer, e.g. LLDPE, will show two or more maxima or at least be distinctly broadened in comparison with the curves for the individual fractions.

Ideally, the molecular weight distribution curve for multimodal polymers of the invention will show two distinct maxima.

For example, if a polymer is produced in a sequential multistage process, utilising reactors coupled in series and using different conditions in each reactor, the polymer fractions produced in the different reactors will each have their own molecular weight distribution and weight average molecular weight. When the molecular weight distribution curve of such a polymer is recorded, the individual curves from these fractions are superimposed into the molecular weight distribution curve for the total resulting polymer product, usually yielding a curve with two or more distinct maxima.

In any multimodal LLDPE, there is by definition a lower molecular weight component (LMW) and a higher molecular weight component (HMW). The LMW component has a lower molecular weight than the higher molecular weight component. This difference is preferably at least 5000. Preferably, in a multimodal LLDPE of use in this invention at least one of the LMW and HMW components is a copolymer of ethylene. Further preferably, at least the HMW component is an ethylene copolymer. Further preferably, also the lower molecular weight (LMW) component may be an ethylene copolymer. Alternatively, if one of the components is a homopolymer, then LMW is the preferably the homopolymer.

Alternatively the multimodal LLDPE may comprise other polymer components, e.g. up to 10% by weight of a well known polyethylene prepolymer (obtainable from a prepolymerisation step as well known in the art). In case of such prepolymer, the prepolymer component is comprised in one of LMW and HMW components, preferably LMW component, as defined above.

The term "ethylene copolymer" is used in this context to encompass polymers comprising repeat units deriving from ethylene and at least one other  $C_{4-12}$  alpha olefin monomer. Preferred copolymers are binary and comprise a single comonomer or are terpolymers and comprise two or three comonomers. In any copolymeric HMW component, preferably at least 0.25 mol-%, preferably at least 0.5 mol-%, e.g. at least 1 mol-%, such as up to 10 mol-%, of repeat units derive from the comonomer. Ethylene preferably forms the majority of the HMW component.

The preferred multimodal LLDPE composition is defined further below. Accordingly, the multimodal LLDPE composition may have a density of no more than 940 kg/m<sup>3</sup>, e.g. 905-940 kg/m<sup>3</sup>. The density is preferably 915 kg/m<sup>3</sup> or more. Ideally, the multimodal LLDPE preferably has a density of 915 to 935 kg/m<sup>3</sup>.

The melt flow rate, MFR<sub>2</sub> of the multimodal LLDPE is preferably in the range 0.01 to 20 g/10min, e.g. 0.05 to 10 g/10min, preferably 0.1 to 6.0 g/10min. The MFR<sub>2</sub> is highly preferably in the range of 0.10 to 5 g/10min.

The MFR<sub>21</sub> of the multimodal LLDPE may be in the range 5 to 500, preferably 10 to 200 g/10min.

The Mw of the multimodal LLDPE, may be in the range 100,000 to 300,000, preferably 150,000 to 270,000. The Mw/Mn of the multimodal LLDPE may be in the range 10 to 30, preferably 10 to 25.

The multimodal LLDPE, may be formed from ethylene along with at least one  $C_{4-12}$  alpha-olefin comonomer, e.g. 1-butene, 1-hexene or 1-octene. Preferably, the multimodal LLDPE, is a binary copolymer, i.e. the polymer contains ethylene and one comonomer, or a terpolymer, i.e. the polymer contains ethylene and two or three comonomers. Preferably, the multimodal LLDPE, comprises an ethylene hexene copolymer, ethylene octene copolymer or ethylene butene copolymer. The amount of comonomer present in the multimodal LLDPE, is preferably 0.5 to 12 mol %, e.g. 2 to 10% mole relative to ethylene, especially 4 to 8% mole.

As stated above a multimodal LLDPE comprises at least a LMW component and a HMW component.

The LMW component of LLDPE preferably has a MFR<sub>2</sub> of at least 50, preferably 50 to 3000 g/10 min, more preferably at least 100 g/10 min. The molecular weight of the low molecular weight component should preferably range from 20,000 to 50,000, e.g. 25,000 to 40,000.

The density of the lower molecular weight component may range from 930 to 980 kg/m<sup>3</sup>, e.g. 940 to 970 kg/m<sup>3</sup>, more preferably 945 to 955 kg/m<sup>3</sup> in the case of copolymer and 940 to 975 kg/m<sup>3</sup>, especially 960 to 972 kg/m<sup>3</sup> in the case of homopolymer.

The lower molecular weight component preferably forms from 30 to 70 wt %, e.g. 40 to 60% by weight of the multimodal LLDPE with the higher molecular weight component forming 70 to 30 wt %, e.g. 40 to 60% by weight.

The higher molecular weight component has a lower MFR<sub>2</sub> and a lower density than the lower molecular weight component.

The higher molecular weight component has preferably an MFR<sub>2</sub> of less than 1 g/10 min, preferably less than 0.5 g/10 min, especially less than 0.2 g/10min, and a density of less than 915 kg/m<sup>3</sup>, e.g. less than 910 kg/m<sup>3</sup>, preferably less

than 905 kg/m<sup>3</sup>. The Mw of the higher molecular weight component may range from 100,000 to 1,000,000, preferably 250,000 to 500,000.

#### Preparation of polymer

The multimodal LLDPE can be any conventional, e.g. commercially available, polymer composition. Alternatively, suitable polymer compositions can be produced in a known manner according to or analogously to conventional polymerisation processes described in the literature of polymer chemistry.

Unimodal LLDPE, is preferably prepared using a single stage polymerisation, e.g. slurry or gas phase polymerisation, preferably a slurry polymerisation in slurry tank or, more preferably, in loop reactor in a manner well known in the art. As an example, a unimodal LLDPE can be produced e.g. in a single stage loop polymerisation process according to the principles given below for the polymerisation of low molecular weight fraction in a loop reactor of a multistage process, naturally with the exception that the process conditions (e.g. hydrogen and comonomer feed) are adjusted to provide the properties of the final unimodal polymer.

Multimodal (e.g. bimodal) polymers can be made by mechanical blending two or more, separately prepared polymer components or, preferably, by in-situ blending in a multistage polymerisation process during the preparation process of the polymer components. Both mechanical and in-situ blending are well known in the field.

Accordingly, preferred multimodal LLDPEs, are prepared by in-situ blending in a multistage, i.e. two or more stage, polymerization or by the use of two or more different polymerization catalysts, including multi- or dual site catalysts, in a one stage polymerization.

Preferably the multimodal LLDPE, is produced in at least two-stage polymerization using the same catalyst, e.g. a single site or Ziegler-Natta catalyst. Thus, for example two slurry reactors or two gas phase reactors, or any combinations thereof, in any order can be employed. Preferably however, the multimodal polymer, e.g. LLDPE, is made using a slurry polymerization in a loop reactor followed by a gas phase polymerization in a gas phase reactor.

A loop reactor - gas phase reactor system is marketed by Borealis as a BORSTAR reactor system. Any multimodal polymer, e.g. LLDPE, present is thus preferably formed in a two stage process comprising a first slurry loop polymerisation followed by gas phase polymerisation.

The conditions used in such a process are well known. For slurry reactors, the reaction temperature will generally be in the range 60 to 110° C. (e.g. 85-110° C.), the reactor pressure will generally be in the range 5 to 80 bar (e.g. 50-65 bar), and the residence time will generally be in the range 0.3 to 5 hours (e.g. 0.5 to 2 hours). The diluent used will generally be an aliphatic hydrocarbon having a boiling point in the range -70 to +100° C. In such reactors, polymerization may if desired be effected under supercritical conditions. Slurry polymerisation may also be carried out in bulk where the reaction medium is formed from the monomer being polymerised.

For gas phase reactors, the reaction temperature used will generally be in the range 60 to 115° C. (e.g. 70 to 110° C.), the reactor pressure will generally be in the range 10 to 25 bar, and the residence time will generally be 1 to 8 hours. The gas used will commonly be a non-reactive gas such as nitrogen or low boiling point hydrocarbons such as propane together with monomer (e.g. ethylene).

Preferably, the lower molecular weight polymer fraction is produced in a continuously operating loop reactor where ethylene is polymerised in the presence of a polymerization

catalyst as stated above and a chain transfer agent such as hydrogen. The diluent is typically an inert aliphatic hydrocarbon, preferably isobutane or propane.

The higher molecular weight component can then be formed in a gas phase reactor using the same catalyst.

Where the higher molecular weight component is made second in a multistage polymerisation it is not possible to measure its properties directly. However, the skilled man is able to determine the density, MFR<sub>2</sub> etc of the higher molecular weight component using Kim McAuley's equations. Thus, both density and MFR<sub>2</sub> can be found using K. K. McAuley and J. F. McGregor: On-line Inference of Polymer Properties in an Industrial Polyethylene Reactor, AIChE Journal, June 1991, Vol. 37, No, 6, pages 825-835.

15 The density is calculated from McAuley's equation 37, where final density and density after the first reactor is known.

20 MFR<sub>2</sub> is calculated from McAuley's equation 25, where final MFR<sub>2</sub> and MFR<sub>2</sub> after the first reactor is calculated. The use of these equations to calculate polymer properties in multimodal polymers is common place.

25 The multimodal LLDPE may be made using any conventional catalyst, such as a chromium, single site catalyst, including metallocenes and non-metallocenes as well known in the field, or Ziegler-Natta catalysts as is also known in the art. The preferred choice is any conventional Ziegler Natta catalyst. Such an LLDPE is called a znLLDPE herein.

In case of znLLDPE the polyethylene polymer composition is manufactured using Ziegler-Natta catalysis. Preferred 30 Ziegler-Natta catalysts comprise a transition metal component and an activator. The transition metal component comprises a metal of Group 4 or 5 of the Periodic System (IUPAC) as an active metal. In addition, it may contain other metals or elements, like elements of Groups 2, 13 and 17.

35 Preferably, the transition metal component is a solid. More preferably, it has been supported on a support material, such as inorganic oxide carrier or magnesium halide. Examples of such catalysts are given, among others in WO 95/35323, WO 01/55230, WO 2004/000933, EP 810235 and WO 99/51646.

In a very preferable embodiment of the invention the polyethylene composition is produced using a Ziegler Natta catalyst disclosed in WO 2004/000933 or EP-A-0688794.

40 Conventional cocatalysts, supports/carriers, electron donors etc can be used.

#### Films

The films of the invention can be multilayer films or monolayer films. In its simplest embodiment, the present 50 invention covers a collation shrink film which is a monolayer film comprising a multimodal LLDPE as herein described as the major component. The monolayer film may simply consist essentially of the multimodal LLDPE. Any film might also contain a mixture of multimodal LLDPE's of the invention.

55 The term consist essentially of is used in this context to indicate that the only polyolefin present is the multimodal LLDPE. The film may however contain standard polymer additives as described below, possibly added via a masterbatch. The levels of these additives are low, typically below 3 wt %.

60 The monolayer film can be formed by extrusion of the necessary polymer to form the film. Monolayer films might also be produced by coextrusion of the same material into separate layers. Such layers become essentially indistinguishable after extrusion. It will be appreciated that the films of the invention might comprise a blend of two or more different multimodal LLDPE's.

It is preferred however if the multimodal LLDPE is blended with other components in order to form the films of the invention. Ideally, therefore the films of the invention are monolayer films in which the multimodal LLDPE of the invention forms the major component or are multilayer films which comprise multimodal LLDPE as the major component. This might be present in one layer of a multilayer film or in more than one layer of a multilayer film.

In addition to the multimodal LLDPE, the films of the invention might contain LDPE (low density polyethylene) or a unimodal LLDPE especially one made using metallocene type catalysis. The films might also contain a very low density polyethylene, i.e. an ethylene with C3-12 alpha olefin copolymer having a density of 900 kg/m<sup>3</sup> or less. These polymers are preferably metallocene produced. Preferred very low density polyethylenes have a density of 850 to 900 kg/m<sup>3</sup>, such as 860 to 895 kg/m<sup>3</sup>. They may have an MFR<sub>2</sub> of 0.4 to 3 g/10 min.

It is preferred if the films of the invention are free of any high density polyethylene, i.e. a polyethylene homopolymer or copolymer with a C3-12 alpha olefin having a density of more than 940 kg/m<sup>3</sup>.

It is also preferred if the films of the invention are free of any ethylene (meth)acrylate polymers.

In a further preferred embodiment the films of the invention are free of LDPE. It is believed that the presence of LDPE in the films of the invention might impart poor stretch and poor mechanical properties to the film. Moreover, LDPE does not assist the shrinkage properties of the film.

Films of the invention may also be free of the very low density polyethylene defined above.

It is especially preferred therefore if the films of the invention are free of HDPE, LDPE and acrylates. Thus, the films preferably consist essentially of the multimodal LLDPE, an optional unimodal LLDPE and an optional very low density polyethylene component.

Unimodal LLDPE's are LLDPEs which have a single peak in the GPC curve and which are therefore produced in a single polymerisation step. Unimodal LLDPEs are preferably metallocene produced, i.e. they are synthesised using metallocene catalysis. This gives characteristic features to the polymer such as narrow Mw/Mn, even comonomer distribution (observable under TREF) and so on. These polymers will be called unimodal mLLDPE's herein.

As used herein, the unimodal LLDPE polymer is an ethylene copolymer having a density of 940 kg/m<sup>3</sup> or less. Preferred unimodal LLDPE's may have a density of 905-940 kg/m<sup>3</sup>, more preferably 910 to 937 kg/m<sup>3</sup>, e.g. 935 kg/m<sup>3</sup> or below. In one preferable embodiment even densities of 925 kg/m<sup>3</sup> or below are highly feasible.

The unimodal LLDPE is formed from ethylene along with at least one C4-12 alpha-olefin comonomer, e.g. 1-butene, 1-hexene or 1-octene. Preferably, the unimodal LLDPE is a binary copolymer, i.e. the polymer contains ethylene and one comonomer, or a terpolymer, i.e. the polymer contains ethylene and two or three, preferably two, comonomers. Preferably, the unimodal LLDPE comprises an ethylene hexene copolymer, ethylene octene copolymer, ethylene butene copolymer or a terpolymer of ethylene with 1-butene and 1-hexene comonomers. The amount of comonomer present in the unimodal LLDPE is preferably 0.5 to 12 mol %, e.g. 2 to 10% mole, especially 4 to 8% mole.

The MFR<sub>2</sub> of unimodal LLDPE's is preferably in the 0.01 or more, preferably 0.1 to 20 g/10min, e.g. 0.2 to 10, preferably 0.5 to 6.0, e.g. 0.7 to 4.0 g/10min.

The unimodal LLDPE has preferably a weight average molecular weight (Mw) of 100,000-250,000, e.g. 110,000-160,000.

The unimodal LLDPE polymers preferably possess a narrow molecular weight distribution. The Mw/Mn value is preferably 2 to 8, e.g. 2.2 to 4.

Unimodal LLDPEs are well known commercial products. The invention especially covers therefore a collation shrink film comprising multimodal LLDPE, and a unimodal LLDPE.

It is preferred if films of the invention are multilayered. Multilayer films are preferably formed from at least three layers, such as 3 layers, 5 layers or 6 layers. Films preferably comprise therefore at least layers A, B and C.

It is preferred if two or more of the layers in the films of the invention comprise a multimodal LLDPE as hereinbefore defined. It is especially preferred if at least layer (A) and layer (B) of the film comprise a multimodal LLDPE.

The (A) layer of the film is preferably an external layer.

It is preferably involved in sealing of the film (to itself). Said layer (A) preferably comprises at least a multimodal LLDPE, in particular a multimodal Ziegler Natta LLDPE. Ideally, this layer is a blend of that multimodal LLDPE with a unimodal LLDPE in particular a mLLDPE. These single site LLDPEs impart excellent sealing behaviour to the films. The (A) layer may also be a blend of the multimodal LLDPE component and a very low density polyethylene as herein described.

Said layer (B) preferably comprises, e.g. consist of a multimodal LLDPE. Said layer (C) preferably comprises the same structure as layer (A). Preferred films of the invention are therefore ABA type films.

#### Film layers

The term "consisting essentially of" used below in relation to film layer materials is meant to exclude only the presence of other polyolefin components, preferably other polymers. Thus said term does not exclude the presence of additives, e.g. conventional film additives, i.e. each layer independently may contain conventional film additives such as antioxidants, UV stabilisers, acid scavengers, nucleating agents, anti-blocking agents, slip agents etc as well as polymer processing agent (PPA) and so on.

Films of the invention preferably comprise layers (A) and (B) below, especially layers (A), (B) and (C) below.

#### Layer (A)

Accordingly, in a first preferable embodiment (i) of the invention, said layer (A) comprises a mixture of a multimodal LLDPE and unimodal LLDPE or very low density polyethylene. In this embodiment (i) a layer (A) preferably comprises 40-75 w % of multimodal LLDPE, more preferably 40 to 70% of multimodal LLDPE. Layer (A) of the embodiment (i) preferably comprises 25-60 wt % unimodal LLDPE or very low density polyethylene, more preferably 30-60 wt %. The use of a 50/50 wt % split of multimodal and unimodal LLDPE or very low density polyethylene is especially preferred here. Layer (A) preferably consists essentially of these components.

#### Layer (B)

Layer (B) preferably comprises at least 50 wt %, preferably at least 60 wt %, more preferably at least 70 wt % of a multimodal LLDPE. In some embodiments even about 80 wt % or more of multimodal LLDPE is preferred. Multimodal LLDPE is preferably a multimodal zLLDPE. Preferably said layer (B) consists of a multimodal LLDPE polymer(s). It may therefore comprise a blend of two multimodal LLDPE's or a single multimodal LLDPE.

#### Layer (C)

## 11

Said layer (C) may have a polymer composition as described in relation to layer (A) above. Preferably layers (A) and (C) are identical in a ABA type film structure.

The film thickness distribution (%) of a ABC layer film is preferably 20 to 40%/2060%/20-40% of the total film thickness (100%).

In a further preferred embodiment, the films of the invention comprise at least five/six layers, preferably in the following order:

- (i) a first outer layer (A),
- (ii) a second outer layer (B),
- (iii) a first inner layer (C),
- (iv) a second inner layer (C),
- (v) a third outer layer (B) and
- (vi) a fourth outer layer (A)

This film is preferably formed from two identical ABC type films and it can be argued that the centre C layers merge to become one (and hence a 5 layer construction). For an ABCCBA film structure the thickness of the layers may conform to 7.5-27.5%/15-35%/525%/15-35%/7.5-27.5%, wherein the total film thickness is 100% and the amount of core layer is the sum of two layers (C).

In an ABCCBA structure it is preferred if the (C) layers are not the same as the (A) layers. In particular, the (C) layers can comprise a very low density polyethylene as hereinbefore defined.

Each A, B or C layer may independently have a composition as hereinbefore defined. Ideally, the ABCCBA film is formed from two identical ABC films laminated together via their (C) layers.

#### Film preparation

Collation shrink films are produced by extrusion through an annular die with a pressure difference applied to blow the extruded cylinder into a film and achieve the desired orientation within the film, i.e. to build a stress into the cooled film. Heat treatment results in stress relaxation and, as a result, shrinkage. Most of the shrinkage occurs while the film is at its hottest (generally ca. 120-130° C.) during the heat treatment; however the film continues to shrink as it cools. These are referred to as the hot shrink force and the cold shrink force respectively and for a polymer to function adequately as the base material for a collation shrink film it should meet the different requirements (in terms of melt strength, cold strength and other mechanical properties) of the hot shrink, cold shrink and post-shrinkage stages.

Collation shrink films of the invention have a particularly beneficial cold shrink force. The high cold shrink forces provide excellent holding properties, i.e. they serve to stabilize the shrink-wrapped product. Moreover, the shrunk film has mechanical properties which are improved relative to conventional shrink films, especially at very low temperatures. As a result the shrink films of the invention are especially suited for use in packaging products which will be exposed to low temperatures during transportation or storage.

Thus the films of the invention exhibit the following advantageous properties:

- high cold shrink force, leading to better holding by the shrunk film of objects packaged by it;
- improved mechanical properties for the shrink film, allowing more demanding (e.g. sharp edged) products to be shrink wrapped and/or allowing thinner films to be used (and hence allowing the amount of polymer wrapping to be reduced); and
- a glossy or transparent optics.

For film formation using polymer mixtures the different polymer components (e.g. within layers (A), (B) and

## 12

optional (C)) are typically intimately mixed prior to extrusion and blowing of the film as is well known in the art. It is especially preferred to thoroughly blend the components, for example using a twin screw extruder, preferably a counter-rotating extruder prior to extrusion and film blowing.

The films of the invention are uniaxially oriented. That means that are stretched in a single direction, the machine direction.

10 The preparation of a uniaxially oriented multilayer film of the invention comprises at least the steps of forming a layered film structure and stretching the obtained multilayer film in a draw ratio of at least 1:3.

Typically the compositions providing the layers of the 15 film will be blown i.e. (co)extruded at a temperature in the range 160° C. to 240° C., and cooled by blowing gas (generally air) at a temperature of 10 to 50° C. to provide a frost line height of 1 or 2 to 8 times the diameter of the die. The blow up ratio should generally be in the range 1.2 to 6, 20 preferably 1.5 to 4.

The obtained film is subjected to a subsequent stretching step, wherein the film is stretched in the machine direction. Stretching may be carried out by any conventional technique using any conventional stretching devices which are well known to those skilled in the art.

25 Preferably for ABCCBA type film structures, said film can advantageously be prepared first by coextruding compositions forming the layers (B), (C) and (A) through an annular die, blowing by blown extrusion into a tubular film 30 to form a bubble. The formed bubble is then collapsed e.g. in nip rolls to form said film where layers (C) are contacted inside/inside, i.e. ABC/CBA. Alternatively, the coextruded bubble may be collapsed and split into two films. The two films can then be stretched separately in a winding machine 35 (2×ABC films).

40 Stretching is preferably carried out at a temperature in the range 70-90° C., e.g. about 80° C. Any conventional stretching rate may be used, e.g. 2 to 40%/second.

The film is stretched only in the machine direction to be 45 uniaxial. The effect of stretching in only one direction is to uniaxially orient the film.

The film is stretched at least 3 times, preferably 3 to 10 times, its original length in the machine direction. This is stated herein as a draw ratio of at least 1:3, i.e. "1" represents 50 the original length of the film and "3" denotes that it has been stretched to 3 times that original length. Preferred films of the invention are stretched in a draw ratio of at least 1:4, more preferably between 1:5 and 1:8, e.g. between 1:5 and 1:7. An effect of stretching (or drawing) is that the thickness 55 of the film is similarly reduced. Thus a draw ratio of at least 1:3 preferably also means that the thickness of the film is at least three times less than the original thickness.

Blow extrusion and stretching techniques are well known in the art, e.g. in EP-A-299750.

55 The film preparation process steps of the invention are known and may be carried out in one film line in a manner known in the art. Such film lines are commercially available.

The films of the invention typically have a starting (or original) thickness of 400 µm or less, preferably 40 to 300 µm, more preferably 50 to 250 µm an prior to the stretching step.

60 After stretching, the final thickness of the uniaxially oriented films, of the invention is typically 50µm or less, preferably 10 to 50µm, more preferably 15 to 40 µm, still more preferably 20 to 38 µm, e.g. 25 to 38 µm, especially 28 to 32 µm.

Film Properties

When subjected to heat, such as in the shrink tunnel, it is preferred if the films of the invention contract in the machine direction by between 40 and 85% such as 50 to 80%, such as 60 to 75%. This shrinkage ratio represents the total shrink of the film, i.e. that which occurs during the heating process in the tunnel/oven and the shrinkage which occurs during the cooling process.

It is preferred if the film of the invention shrinks by at least 50% in the machine direction even when exposed to heat of 170° C. or less. It is preferred if the films of the invention shrink by at least 50% in the machine direction at temperatures of between 80 and 160° C., such as 90 to 150° C.

Shrink in the transverse direction can be up to 10%. Ideally transverse direction shrinkage is up to 10%, especially in the temperature range of 90 to 170° C.

The films of the invention preferably have high stiffness before the shrink process. Higher stiffness allows the collation shrink film to be easily handled. Film stiffness before shrinkage may be 700 to 1000 MPa.

The material may have high penetration energy to withstand sharp objects. Puncture resistance values may be of the order of 22 J/mm before shrinkage.

Bundling force or cold shrink force is preferably above 2 N in the machine direction.

The films of the invention preferably have a haze value of less than 20 before shrinkage.

#### Binding tape

The invention requires the use of a binding tape. The binding tape is a comparatively thin strip of film that is used to wrap around the object as described herein. The tape will be thinner in width than the height of any containers within the object being packaged. The binding tape can be any uniaxially oriented film (oriented in the machine direction). It must be stretched by at least 3 times its length during the orientation process. More preferably, the binding tape may be a uniaxially oriented film as described above for the collation shrink film. Ideally therefore, the binding tape is a uniaxially oriented film comprising a multimodal LLDPE.

Ideally of course, the binding tape is formed from exactly the same material as the collation shrink film. The binding tape is therefore preferably simply a thin strip of film cut off from the main collation shrink film.

The thickness of the binding tape might vary depending on the size of the object being packaged but is generally of the same dimensions of the collation shrink film. The binding tape of the invention typically has a starting (or original) thickness of 400 µm or less, preferably 40 to 300 µm, more preferably 50 to 250 µm prior to the stretching step.

After stretching, the final thickness of the uniaxially oriented films, of the invention is typically 50 µm or less, preferably 10 to 50 µm, more preferably 15 to 40 µm, still more preferably 20 to 38 µm, e.g. 25 to 38 µm, especially 28 to 32 µm.

The width of the binding tape might vary depending on the size of the object being packaged. Widths from 0.5 cm to 20 cm might be appropriate, such as 1 to 18 cm, preferably 2 to 16 cm, especially 4 to 14 cm, e.g. 6 to 12 cm. Preferred binding tapes might be 10 to 70% of the height of the containers in the object, such as 20 to 60%.

It will be obvious that the length of the binding tape must be sufficient to be wrapped around the whole of the object with a degree of overlap to allow the ends of the binding tape to be sealed to each other.

The binding strip is preferably sealed before the collation shrink film is applied. Sealing can be effected using sealing bars.

#### Collation Shrink Process

5 The collation shrink wrapping process is a conventional one and the steps of that process are well known to the skilled person. The collation shrink film of the invention can be wrapped around an object in a conventional manner. The collation shrink film is typically supplied in a large roll in its 10 stretched form. Film is dispensed from the roll, cut and placed over the object to be wrapped. The film can be cut into appropriate lengths as it is dispensed from the roll.

Generally the object to be collation shrink wrapped will 15 be present on a conveyor belt or other conveying means. The wrapping process is a continuous process so the conveyor will contain a plurality of objects to be wrapped with each being wrapped in turn.

As each object moves along the conveyor, the collation shrink film is moved over the top of the object and then 20 wrapped over it, down two of its opposite sides and underneath it using conventional equipment. The ends of the film are therefore brought together and contacted underneath the object. These ends form a seal during the later shrink process or can be sealed using sealing bars as described later.

The other two sides of the object remain open but the film 25 used will be wider than the object so that there will be film protruding around the open ends of the object. In the shrink tunnel, the protruding film folds in to wrap the open ends, although there is still a hole in the center of the open ends, 30 as is well known in the art.

It will be appreciated that in the wrapping process, two 35 sides of the object are covered and two ends of the object remain open. It is preferred if the shorter side of any object remains open and the longer side covered. Thus, when packaging an object comprising a 2x3 arrangement of containers, the open ends are placed on the two container side with the covered side along the 3 container side. Obviously, if the object is a square then there is no shorter side and it doesn't matter which side is which.

40 The machine direction in this 2x3 type example is parallel to the 2 container side. When the film shrinks it compresses the 2 containers in each row together. There is less bundling force compressing the containers along the 3 container axis.

In the present invention, a binding tape is also used to 45 solve this problem. This tape might be supplied separately to the main collation shrink film or it may be part of the shrink film which is cut off to form the binding tape.

Before the main collation shrink film is wrapped around the object, the binding tape is wrapped around the object. It 50 is necessary to wrap the binding tape such that when it shrinks in its machine direction, it provides bundling force in the transverse direction of the main collation shrink film. One of the problems with the collation shrink films of this invention is a lack of bundling force in the transverse direction. 55 By using a binding tape, we solve this problem.

A binding tape can therefore be applied around the object before the collation shrink film such that it is under the collation shrink film in the final object. The two ends of the binding tape need to overlap and remain in contact to allow 60 a seal in the binding tape to form. The seal must be formed before the main collation shrink film is applied. Sealing is effected conventionally using heat.

When the binding tape shrinks, it too preferably shrinks 65 mostly in its machine direction. The tape is oriented such that the machine direction shrinkage of the binding tape effectively provides bundling force in the transverse direction of the main collation shrink film. In our example of the

## 15

2x3 containers, the tape can be wrapped around the sides of the object (as opposed to the base or the top of the object). When it shrinks therefore it provides compressive (bundling force) down the 3 container axis. It compresses the three containers in each column together. The binding tape will also partially cover the open end of the object. This is generally illustrated in FIG. 3. It is therefore preferred if the binding tape is wrapped around the sides of the object, i.e. horizontal rather than vertical.

Once the binding tape and collation shrink film have been applied, the wrapped object is heated in some fashion to enable the collation shrink process. Ideally, the wrapped object is passed through a heat tunnel in order to shrink the film around the object and to shrink the binding tape. Preferably this process also seals the collation shrink film to itself underneath the object.

Current shrink tunnels typically employ temperatures of 180 to 210° C. This exposes therefore the material being packaged to high temperature albeit for a short period of time. It is perceived however, that these high temperatures are required to enable the necessary collation shrinkage properties and to effect a seal of the film underneath the object.

It is a major benefit of the use of the collation shrink films of the invention that commercially relevant levels of machine direction shrinkage can be achieved at much lower temperatures. As the binding tape is also a uniaxial oriented film ideally of a multimodal LLDPE, it too shrinks at low temperature.

The temperature to which the collation shrink films of this invention are exposed may be up to 170° C., preferably up to 160° C., such as 80 to 150° C. Ideally the temperature is in the range of 90 to 140° C.

Note of course, that what matters here is the temperature which the film experiences. In order to make sure that the film experiences a particular temperature, it may be that the shrink tunnel has to be a little warmer than that temperature. In terms of the temperatures experience by the film itself, we have observed useful shrink properties when the actual film temperature is 140° C. or less such as 80 to 135° C., especially 90 to 130° C.

For the targeted machine direction oriented films of this invention, the tunnel temperature could be reduced to 130-170° C. for example, in order to make sure that the collation shrink films within the tunnel experience the temperatures mentioned above.

Low shrinkage temperatures, might however lead to poor film sealing in the collation shrink film. It may therefore be necessary to use sealing bars to effect a seal of the two ends of the collation shrink film of the invention. This may be carried out before the object is exposed to shrink temperatures.

The object may spend up to 1 min in the heated zone in order to ensure that the collation shrink wrapping occurs, such as 20 to 30 seconds.

As can be seen from FIG. 3, the binding tape will generally provide bundling force horizontally. The collation film will generally provide bundling force vertically.

## Applications

The collation shrink films of the invention are preferably used in the wrapping of household, food, healthcare or beverage products, in particular products that are packaged in containers such as bottles, cans, tubs and the like. Whenever a product is shipped in numerous essentially identical containers, the use of collation shrink film is useful to prevent damage to the products and keep the product secure

## 16

during transport. The most common application is therefore in the beverage transportation market.

It will be appreciated that the collation shrink film might also be used to wrap industrial products such as chemicals and the like.

The invention will now be described with reference to the following non-limiting examples and figures.

FIG. 1 shows the relative machine direction shrinkage properties of the films of the invention relative to a non oriented reference film at various different temperatures.

FIG. 2 shows the cold shrink force as a function of shrink rate at different temperatures (100-200° C.).

FIG. 3 is a depiction of an object collation shrink wrapped using a binding tape and film as claimed herein.

## 15 Determination methods

Density of the materials is measured according to ISO 1183:1987 (E), method D, with isopropanol-water as gradient liquid. The cooling rate of the plaques when crystallising the samples was 15 ° C/min. Conditioning time was 16 hours.

## 20 Melt Flow Rate (MFR) or Melt Index (MI)

The melt flow rate (MFR) is determined according to ISO 1133 and is indicated in g/10 min. The MFR is an indication of the melt viscosity of the polymer. The MFR is determined at 190° C. for PE and at 230 ° C. for PP. The load under which the melt flow rate is determined is usually indicated as a subscript, for instance MFR<sub>2</sub> is measured under 2.16 kg load, MFR<sub>5</sub> is measured under 5 kg load or MFR<sub>21</sub> is measured under 21.6 kg load.

## 30 Molecular weights, molecular weight distribution, Mn, Mw, MWD

The weight average molecular weight Mw and the molecular weight distribution (MWD =Mw/Mn wherein Mn is the number average molecular weight and Mw is the weight average molecular weight) is measured by a method based on ISO 16014-4:2003. A Waters 150CV plus instrument, equipped with refractive index detector and online viscosimeter was used with 3 xHT6E styragel columns from Waters (styrene-divinylbenzene) and 1,2,4-trichlorobenzene (TCB, stabilized with 250 mg/L 2,6-Di tert butyl-4-methylphenol) as solvent at 140 ° C. and at a constant flow rate of 1 mL/min. 500 µL of sample solution were injected per analysis. The column set was calibrated using universal calibration (according to ISO 16014-2:2003) with 10narrow MWD polystyrene (PS) standards in the range of 1.05 kg/mol to 11 600 kg/mol. Mark Houwink constants were used for polystyrene and polyethylene (K: 19×10<sup>-3</sup> dL/g and a: 0.655 for PS, and K: 39×10<sup>-3</sup> dL/g and a: 0.725 for PE). All samples were prepared by dissolving 0.5 -3.5 mg of polymer in 4 mL (at 140 ° C.) of stabilized TCB (same as mobile phase) and keeping for 2 hours at 140 ° C. and for another 2 hours at 160 ° C. with occasional shaking prior sampling in into the GPC instrument.

55 Comonomer Content (% wt and % mol) was determined by using <sup>13</sup>C-NMR. The <sup>13</sup>C-NMR spectra were recorded on Bruker 400 MHz spectrometer at 130 ° C. from samples dissolved in 1,2,4-trichlorobenzene/benzene-d<sub>6</sub> (90/10 w/w). Conversion between % wt and % mol can be carried out by calculation.

## 60 Haze is measured according to ASTM D 1003.

Cold shrink forces have been measured according to standard ISO 14616:1997 in Machine (MD) direction in the following way. Specimens of 15 mm width and 115 mm length are cut out from the film sample MD. The samples are 65 tightly mounted into the jaws of the load cell in such a way that the distance between the jaws is 100 mm and the actual force is zero. The samples are then exposed to hot air at

given temperature. After closing the chamber the shrinkage temperature is reached at the maximum force. This is recorded and it represents the hot shrink force. The hot air chamber is removed after force has reduced 15-30% from maximum while continuing to record the force. The maximum force is again recorded and this second maximum represents the cold shrink force.

## EXAMPLE 1

Two 25 micron uniaxially stretched films were produced from two different multimodal LLDPEs. Grade 1 was a multimodal Ziegler Natta linear low density polyethylene having a density of 923 kg/m<sup>3</sup> and an MFR<sub>2</sub> of 0.4 g/10min. Grade 2 is a multimodal Ziegler Natta linear low density polyethylene having a density of 931 kg/m<sup>3</sup> and an MFR<sub>2</sub> of 0.2 g/10min.

The inventive films were made in a first step on a blown film line at a thickness of 150µm, BUR 1:3 and die gap 1.4 mm. The film structure is a monolayer film consisting of Grade 1 or Grade 2 (IE1 or IE2 respectively).

The film is then stretched on an MDO unit with a stretch ratio of 6 at a temperature of ~110° C. This is done by unwinding the film and feeding it into the MDO unit. First the heating rolls get the film to up to a temperature of ~110° C., then the film is stretched in between the stretching rolls due to 6 times higher speed of the second stretching roll over the first one. In an annealing and cooling step the orientation in the film is fixed.

This film was compared to a 30 micron non oriented monolayer film formed from a blend of multimodal znLLDPE (45wt % of density 931 kg/m<sup>3</sup> and MFR<sub>2</sub> 0.2 g/10min)/HDPE (40wt % of density 958 kg/m<sup>3</sup> and MFR<sub>2</sub> of 0.7 g/10min) and LDPE (15 wt % of density 920 kg/m<sup>3</sup> and MFR<sub>2</sub> of 0.3 g/10min).

## Shrinkage in oil:

Comparative determination of shrinkage was performed in oil according to internal Borealis method. 50mm×50mm samples are placed in oil (Polydimethylsiloxan) at given temperature for 10 seconds. After this the samples are removed, and conditioned at room temperature for 1 hour. Finally the shrinkage, i.e. change in dimension is measured. Results are presented in table 1. Shrinkage values are calculated as:

$$\text{Shrinkage} = (L_0 - L_m) * 100 / L_0$$

wherein L<sub>0</sub> is the original length (i.e. 50 mm), and L<sub>m</sub> is the length measured after thermal exposure.

If the measured value increases (e.g. in the TD direction), then shrinkage is negative.

| Shrink Temperature (in Oil) | Parameter       | Unit | Non oriented film |          |      |
|-----------------------------|-----------------|------|-------------------|----------|------|
|                             |                 |      | Film IE1.         | Film IE2 |      |
| 80° C.                      | Length Md After | mm   | 50                | 46.3     | 45.5 |
| 80° C.                      | Length Td After | mm   | 50                | 50.2     | 50   |
| 80° C.                      | Shrinkage Md    | %    | 0                 | 7.4      | 9    |
| 80° C.                      | Shrinkage Td    | %    | 0                 | -0.4     | 0    |
| 100° C.                     | Length Md After | mm   | 50                | 39.2     | 37   |
| 100° C.                     | Length Td After | mm   | 50                | 51.6     | 51.2 |
| 100° C.                     | Shrinkage Md    | %    | 0                 | 21.6     | 26   |
| 100° C.                     | Shrinkage Td    | %    | 0                 | -3.2     | -2.4 |
| 120° C.                     | Length Md After | mm   | 48.7              | 9.5      | 12.1 |
| 120° C.                     | Length Td After | mm   | 50                | 53.5     | 52.9 |
| 120° C.                     | Shrinkage Md    | %    | 2.6               | 81       | 75.8 |
| 120° C.                     | Shrinkage Td    | %    | 0                 | -7       | -5.8 |
| 140° C.                     | Length Md After | mm   | 11.5              | 4        | 4    |
| 140° C.                     | Length Td After | mm   | 46.6              | 44.2     | 44   |

-continued

| Shrink Temperature (in Oil) | Parameter    | Unit | Non oriented film |      | Film IE1. | Film IE2 |
|-----------------------------|--------------|------|-------------------|------|-----------|----------|
| 140° C.                     | Shrinkage Md | %    | 77                | 92   | 92        |          |
| 140° C.                     | Shrinkage Td | %    | 6.8               | 11.6 | 12        |          |

10

## EXAMPLE 2

Mechanical data from the films are presented in Table 2 along with further shrink ratio data. Table 2 shows shrink data occurring the shrink force tests. Due to thermic conductivity, the shrinkage is different than at the same temperature in oil.

TABLE 2

| Shrink Temp. | Parameter (MD always) | Unit | Non oriented film |       | Film IE1 | Film IE2 |
|--------------|-----------------------|------|-------------------|-------|----------|----------|
| 100° C.      | Cold Shrink Force     | N    | nd                | 1.86  | 1.93     |          |
| 100° C.      | Shrink Ratio          | %    | nd                | 15.11 | 18.73    |          |
| 120° C.      | Cold Shrink Force     | N    | 0.18              | 2.44  | 2.59     |          |
| 120° C.      | Shrink Ratio          | %    | nd                | 47.78 | 44.63    |          |
| 150° C.      | Cold Shrink Force     | N    | 1.62              | 0.91  | 3.17     |          |
| 150° C.      | Shrink Ratio          | %    | 12.87             | 80.7  | 80.6     |          |
| 180° C.      | Cold Shrink Force     | N    | 2.09              | nd    | nd       |          |
| 180° C.      | Shrink Ratio          | %    | 71.2              | 87.43 | 90.3     |          |
| 200° C.      | Cold Shrink Force     | N    | 2.03              | nd    | nd       |          |
| 200° C.      | Shrink Ratio          | %    | 71.23             | 93.17 | 91.67    |          |

Nd not determined

Shrink ratios % length that the film is shorter after heat application.

35

## EXAMPLE 3

A 24 pack of soft drink cans, carried in a cardboard tray is collation shrink wrapped using the process of the invention. A collation shrink film (IE1) has cut therefrom a 5 cm wide strip of sufficient length to pass around the side of the case of soft drinks. The binding tape is passed around the sides of the soft drinks case and the overlapping ends of the tape are sealed with sealing bars.

Thereafter, a collation shrink film (IE1) is dispensed from a roll and cut to an appropriate length. The film is placed over the soft drinks case with the sealed binding tape and passed down the longer sides of the case and underneath the case using conventional technology. A seal is formed underneath the case using sealing bars.

The whole object is passed into a shrink tunnel for 30 seconds at a temperature of 165° C. The collation shrink film and the binding tape both contract in the machine direction such that those directions are orthogonal.

55

We claim:

1. A process for collation shrink wrapping an object which comprises a plurality of individual containers, comprising:
  - (i) obtaining a binding tape which is a film uniaxially oriented in the machine direction (MD) and wrapping said tape around said object;
  - (ii) sealing the ends of the now wrapped binding tape to form a loop;
  - (iii) obtaining a collation shrink film comprising a multimodal linear low density polyethylene (LLDPE), said collation shrink film being a monolayer stretched film which is uniaxially oriented in the machine direction

60

65

## 19

- (MD) in a draw ratio of at least 1:3 and which has a haze value of less than 20% before shrinkage;
- (iv) wrapping said collation shrink film around said object of step (ii);
- (v) heating said wrapped object of step (iv) to a temperature of 170° C. or less such that the binding tape shrinks in its machine direction and the collation shrink film shrinks by at least 50% in its machine direction.
2. A process as claimed in claim 1, whereas said collation shrink film has a thickness of 15 to 40 microns.

3. A process as claimed in claim 1, wherein said multimodal polyethylene is formed from a lower molecular weight homopolymer and a higher molecular weight copolymer.

4. A process as claimed in claim 1, wherein said collation shrink film is free of HDPE and LDPE.

5. A process as claimed in claim 1, wherein said collation shrink film further comprises a unimodal LLDPE.

6. A process as claimed in claim 1, wherein the binding tape is wrapped around the sides of the object.

7. An object wrapped by a process as described in claim 1.

8. A process as claimed in claim 1, wherein said plurality of individual containers are substantially identical containers.

9. A process for collation shrink wrapping an object which comprises a plurality of individual containers, comprising:

(i) obtaining a binding tape which is a film uniaxially oriented in the machine direction (MD) and wrapping said tape around said object;

(ii) sealing the ends of the now wrapped binding tape to form a loop;

(iii) obtaining a collation shrink film comprising a multimodal linear low density polyethylene (LLDPE), said collation shrink film being a monolayer stretched film which is uniaxially oriented in the machine direction (MD) in a draw ratio of at least 1:3 and which has a haze value of less than 20% before shrinkage;

(iv) wrapping said collation shrink film around said object of step (ii) in such a way that when said binding tape shrinks in its machine direction upon the application of heat, that direction represents substantially the transverse direction for the collation shrink film;

(v) heating said wrapped object of step (iv) to a temperature of 170° C. or less such that the binding tape shrinks in its machine direction and the collation shrink film shrinks by at least 50% in its machine direction.

10. A process for collation shrink wrapping an object which comprises a plurality of individual containers, comprising:

5

10

20

25

30

35

40

45

## 20

(i) obtaining a binding tape which is a film uniaxially oriented in the machine direction (MD) and wrapping said tape around said object;

(ii) sealing the ends of the now wrapped binding tape to form a loop;

(iii) obtaining a collation shrink film comprising a multimodal linear low density polyethylene (LLDPE), said collation shrink film being a monolayer stretched film which is uniaxially oriented in the machine direction (MD) in a draw ratio of at least 1:3 and which has a haze value of less than 20% before shrinkage;

(iv) wrapping said collation shrink film around said object of step (ii) in such a way that when said binding tape shrinks in its machine direction upon the application of heat, that direction represents substantially the transverse direction for the collation shrink film, that direction is perpendicular to the shrinkage of the collation shrink film;

(v) heating said wrapped object of step (iv) to a temperature of 170° C. or less such that the binding tape shrinks in its machine direction and the collation shrink film shrinks by at least 50% in its machine direction.

11. A process for a process for collation shrink wrapping an object which comprises a plurality of individual containers, comprising:

(i) obtaining a collation shrink film comprising a multimodal linear low density polyethylene (LLDPE), said collation shrink film being a monolayer stretched film which is uniaxially oriented in the machine direction (MD) in a draw ratio of at least 1:3 and which has a haze value of less than 20% before shrinkage;

(ii) cutting a binding tape from said collation shrink film;

(iii) wrapping said binding tape around said object and sealing the ends of the now wrapped binding tape to form a loop;

(iv) wrapping at least a part of said remaining collation shrink film around said object; in a direction such that when said binding tape shrinks in its machine direction upon the application of heat, that direction represents substantially the transverse direction for the collation shrink film;

(v) heating said wrapped object of step (iv) to a temperature of 170° C. or less such that the binding tape shrinks by at least 50% in its machine direction and the collation shrink film shrinks by at least 50% in its machine direction.

\* \* \* \* \*